

## UNITED STATES PATENT OFFICE

JACK L. BITTER, OF ELIZABETHTON, AND RICHARD ELSSNER, OF JOHNSON CITY, TENNESSEE, ASSIGNORS TO AMERICAN GLANZSTOFF CORPORATION, OF NEW YORK, N. Y., A CORPORATION OF DELAWARE

## TREATMENT OF ARTIFICIAL FILAMENTS

No Drawing.

Application filed August 29, 1931. Serial No. 560,226.

Our invention relates to an improved process for the production of artificial threads, and more particularly to an improved process for producing thread having even elongation and strength.

In the production of artificial silk, according to the wet spinning process, a cellulosic solution is spun into a suitable coagulating medium and the freshly spun threads are collected on suitable spools. The filled spools are then subjected to several after-treatments, such as washing, desulphurizing, bleaching and drying. It is to be understood, however, that the desulphurizing and bleaching steps may be omitted and our invention is not to be limited to the specific after treatments mentioned since these steps are given merely by way of example.

During the drying process the washed yarn shrinks, and the outer layers of the yarn body will shrink more than those layers adjacent the spool, since the latter shrink against a comparatively unyielding surface. This results in an uneven and poor quality of thread since that portion of the thread will possess a lower elongation and higher strength quality than the other parts of the yarn body. These differences of the physical properties are highly undesirable in the dyeing of woven and knitted goods resulting in the so called shiner or barre effects on the goods.

According to our invention the thread treated in the manner noted above, is twisted on any desirable type of spool, and after more or less spraying, is then subjected to a second drying resulting in the yarn which was adjacent the spool during the first drying will be on the outside of the yarn body during the second drying. Thus the yarn last mentioned have the same opportunity to shrink as did the outer layers of yarn before the twisting operation.

The manner in which our invention may be carried into effect can be well illustrated by the following examples, it being understood that these are given only by way of illustration and can be varied widely without departing from the scope thereof:

*Example 1.*—About 70 grams viscose yarn, 150 denier with 32 filaments, soft lustre, spun

on a perforated, lacquered spool, with a circumference of 230 mm. and length of 130 mm. is washed by drip-washing or vacuum washing and is immediately desulphurized and bleached after which it is dried at a temperature of about 70° C. After conditioning the yarn is twisted on any kind of twisting machine in a room which is kept at about 60-80% humidity. After that time the spool is sprayed and then is placed in a dryer for about from 2-8 hours, at about 70° C. Then the yarn is conditioned once more and wound on cones.

*Example 2.*—About 250 grams viscose yarn, 200 denier, with 40 filaments, high lustre, spun on a corrugated rubber spool with a circumference of 400 mm. and a length of 200 mm. is washed by drip-washing or vacuum washing and is immediately desulphurized and bleached, and is then dried at a temperature of about 70° C. After conditioning the spool is twisted on a top twisting machine in a room where the moisture content is about 60-80%. After that time the spool is sprayed and brought once more to a dryer for about 2-8 hours, at about 70° C. Then the spool is conditioned once more and the yarn wound upon cones.

Having now fully set forth our invention as required by the patent statutes, what we desire to claim is:

1. In a method of treating spooled artificial filaments, and the like the steps of wet-treating, drying, rewetting and redrying, the filaments and the like being rewound onto another holder between the first and second drying.

2. In a method for treating freshly spun spooled artificial filaments the steps of successively drying, twisting, spraying and drying the same.

3. In a method for treating freshly-extruded viscose filaments, the steps of winding on spools, washing and desulphurizing the same, drying, twisting, rewetting and redrying.

4. In a method for producing a yarn with an even contraction and strength, the steps of spooling wet-treating and drying the yarn, rewinding so that the yarn formerly on the

outer side of the holder is on the inside, then rewetting and redrying the yarn.

5. In a process for the production of yarn with even shrinkage, the steps of extruding the yarn, winding it onto spools, wet treating it, rewinding onto other spools so the yarn formerly on the inner side of the spool body is later on the outer side, rewetting and redrying.

6. In a process of the class set forth, the steps of winding freshly-spun artificial yarn upon a spool or the like, desulphurizing, bleaching and otherwise aftertreating it, drying at a temperature of approximately 70°

15 C., twisting onto another spool or the like, rewetting, and redrying over a period of from two to eight hours at a temperature of about 70° C.

7. In a process of the class set forth, the 20 steps of winding freshly-spun artificial yarn upon a spool or the like, desulphurizing, bleaching and otherwise aftertreating it, drying at a temperature of approximately 70° C., conditioning, twisting onto another spool 25 or the like, rewetting, and redrying over a period of from two to eight hours at a temperature of about 70° C.

8. In a process of the class set forth, the 30 steps of winding freshly-spun artificial yarn upon a spool or the like, desulphurizing, bleaching and otherwise aftertreating it, drying at a temperature of approximately 70° C., conditioning, twisting onto another spool or the like, in a room the humidity of which 35 is from 60 to 80%, rewetting, and redrying over a period of from two to eight hours at a temperature of about 70° C.

9. In a process of the class set forth the 40 steps of winding a freshly-spun artificial yarn upon a spool or the like, drying at a relatively high temperature, twisting onto another spool or the like, rewetting, and redrying at a relatively high temperature.

45 In testimony whereof we affix our signatures.

JACK L. BITTER.  
DR. RICHARD ELSSNER.

#### DISCLAIMER

1,867,610.—*Jack L. Bitter, Elizabethton, and Richard Elssner, Johnson City, Tenn.*  
TREATMENT OF ARTIFICIAL FILAMENTS. Patent dated July 19, 1932.  
Disclaimer filed November 10, 1934, by the assignee, *North American Rayon Corporation*.

Hereby disclaims from the scope of claims 1, 4, and 5 of said Letters Patent any method or process other than those in which the artificial filaments or yarn are dried at about 70° C. on each holder or spool and/or in which the artificial filaments or yarn are desulphurized and subsequently twisted and rewound onto the second holder or spool.

[Official Gazette December 4, 1934.]

outer side of the holder is on the inside, then rewetting and redrying the yarn.

5. In a process for the production of yarn with even shrinkage, the steps of extruding the yarn, winding it onto spools, wet treating it, rewinding onto other spools so the yarn formerly on the inner side of the spool body is later on the outer side, rewetting and redrying.

6. In a process of the class set forth, the steps of winding freshly-spun artificial yarn upon a spool or the like, desulphurizing, bleaching and otherwise aftertreating it, drying at a temperature of approximately 70°

15 C., twisting onto another spool or the like, rewetting, and redrying over a period of from two to eight hours at a temperature of about 70° C.

7. In a process of the class set forth, the 20 steps of winding freshly-spun artificial yarn upon a spool or the like, desulphurizing, bleaching and otherwise aftertreating it, drying at a temperature of approximately 70° C., conditioning, twisting onto another spool 25 or the like, rewetting, and redrying over a period of from two to eight hours at a temperature of about 70° C.

8. In a process of the class set forth, the 30 steps of winding freshly-spun artificial yarn upon a spool or the like, desulphurizing, bleaching and otherwise aftertreating it, drying at a temperature of approximately 70° C., conditioning, twisting onto another spool or the like, in a room the humidity of which 35 is from 60 to 80%, rewetting, and redrying over a period of from two to eight hours at a temperature of about 70° C.

9. In a process of the class set forth the 40 steps of winding a freshly-spun artificial yarn upon a spool or the like, drying at a relatively high temperature, twisting onto another spool or the like, rewetting, and redrying at a relatively high temperature.

45 In testimony whereof we affix our signatures.

JACK L. BITTER.  
DR. RICHARD ELSSNER.

#### DISCLAIMER

1,867,610.—*Jack L. Bitter, Elizabethton, and Richard Elssner, Johnson City, Tenn.*  
TREATMENT OF ARTIFICIAL FILAMENTS. Patent dated July 19, 1932.  
Disclaimer filed November 10, 1934, by the assignee, *North American Rayon Corporation*.

Hereby disclaims from the scope of claims 1, 4, and 5 of said Letters Patent any method or process other than those in which the artificial filaments or yarn are dried at about 70° C. on each holder or spool and/or in which the artificial filaments or yarn are desulphurized and subsequently twisted and rewound onto the second holder or spool.

[Official Gazette December 4, 1934.]

## DISCLAIMER

1,867,610.—*Jack L. Bitter, Elizabethton, and Richard Elssner, Johnson City, Tenn.*  
**TREATMENT OF ARTIFICIAL FILAMENTS.** Patent dated July 19, 1932.  
Disclaimer filed November 10, 1934, by the assignee, *North American Rayon Corporation.*

Hereby disclaims from the scope of claims 1, 4, and 5 of said Letters Patent any method or process other than those in which the artificial filaments or yarn are dried at about 70° C. on each holder or spool and/or in which the artificial filaments or yarn are desulphurized and subsequently twisted and rewound onto the second holder or spool.

[*Official Gazette December 4, 1934.*]